

## UNITED STATES PATENT OFFICE

2,303,242

## METAL COATING

Robert R. Tanner, Detroit, and Robert V. Harris,  
Highland Park, Mich., assignors to Parker Rust  
Proof Company, Detroit, Mich.

No Drawing. Application November 19, 1938.  
Serial No. 241,393

## 4 Claims. (Cl. 148—6.5)

This invention relates to the production of paint-holding and corrosion-retarding coatings on ferrous surfaces, and relates more especially to producing such coatings by a simpler and more flexible method than is used at the present time in the rustproofing art.

The usual method of rustproofing articles, preparatory to painting, involves reacting the surface for a period with an aqueous acid phosphate solution whereby a coating of insoluble phosphates is formed on the surface. After the production of the coating, the processing solution remaining on the surface is rinsed off with water and the articles then given a rinse in a hot solution of chromic acid. This final rinse has been found to produce a decided advantage in increasing the rustproofing and paint-holding properties of the coating.

When a phosphate coating is formed according to the described method, a part of the iron from the treated surface is dissolved and becomes a part of the coating as an insoluble phosphate along with the insoluble phosphates of the metal used as the acid phosphate in the processing solution. Therefore, if zinc acid phosphate is used, for example, the coating will be composed of a combination of comparatively insoluble phosphates of zinc and iron.

One function of the chromic acid rinse is to dissolve out a part of the zinc phosphate, leaving a coating that is comparatively richer in iron phosphate because this is the more insoluble of the two.

The final chromic acid rinse, therefore, results in a film on the ferrous article which contains iron phosphate, zinc phosphate, hexavalent chromium, and some trivalent chromium resulting from reduction of some chromic acid caused by its dissolving action.

Before a ferrous article can be processed in phosphate solutions it must be cleaned. This is usually done commercially by washing the surface with a hot alkaline solution followed by a water rinse. The strength of the cleaner as well as the time of washing must be carefully regulated, otherwise the phosphate coating will be formed of objectionably large crystals which are lacking in rustproofing ability and also cause a dulling of paint finishes superposed.

Phosphate solutions of the kind described are usually applied by immersing the object to be treated for a period of time in a heated solution until the desired coating is formed, or the solution is sprayed onto the surfaces to obtain

the coating as the articles pass along on a conveyor.

The object of the present invention is to provide a novel method of treating ferrous surfaces by a simpler means than used with the common phosphate method.

It is a further object to provide a treating solution with which a greater latitude of cleaning conditions can be used without encountering the formation of objectionably large phosphate crystals in the coating.

A still further object lies in the use of a solution which will readily and uniformly wet the surface to be treated, thus insuring the maximum results in rustproofing and paint-holding ability.

These objects are accomplished by combining in one solution both the necessary phosphate in the form of a phosphoric acid and the necessary chromic acid, either as such or as an alkali chromate or dichromate, since the addition of either of these will result in the formation of chromic acid in the presence of the phosphoric acid.

The phosphoric acid and chromic acid should be present under conditions where a definite etching of the metal surface will occur. It is essential that the solution applied be retained permanently on the surface and be not rinsed off or otherwise removed.

Whether or not the solution will etch the metal surface depends both on the concentration of the phosphoric acid and the hexavalent chromium, and on the ratio existing between the two.

It is well known that chromic acid in certain amounts has a decided inhibiting action on the attack of phosphoric acid on ferrous surfaces. Since we desire etching, the correct conditions of the solution must be selected. For example, if a concentration of ortho-phosphoric acid of

.5% is used, a ratio of chromic acid to phosphoric acid of .35 to 1 would not cause etching of metal; therefore, the objects of the invention could not be attained, but if this ratio is reduced to .25 to 1 a definite reaction with the metal occurs result-

ing in a protective film of iron phosphate, trivalent chromium, and possibly some hexavalent chromium which has not been reduced. Any ratio of .25 to 1 or less will therefore result in etching and the formation of the desired products of the reaction.

To give a further example, if a concentration of ortho-phosphoric acid of 4% is used, a ratio of chromic acid to phosphoric acid of .25 to 1 will prevent etching, but a ratio of .15 to 1 allows it to proceed as desired. In speaking of etching,

we mean visible etching. The ratios of phosphoric and chromic should be adjusted so that visible etching of the surface is obtained.

In carrying out the process the metal to be treated is first cleaned by any suitable means. Such methods as solvent wiping, or vapor degreasing are usually employed for small articles or where there is a limited amount of production. Alkali cleaning is ordinarily adopted for production lines where auto bodies or sheet metal parts, or similar large objects are to be treated. In this case, the cleaning operation is followed by a water rinse to remove the alkali.

Large objects such as structural members of buildings, in addition to having the grease removed, usually have considerable loose scale and rust and this also must be removed. After the cleaning operation the metal is ready to receive the treatment of the present invention.

If there is any residual grease or oil on the surface it may be difficult to readily obtain uniform wetting and so in order to avoid poor results it is usually advisable to incorporate in the treating solution a wetting agent. There is a wide selection of these materials suitable for the purpose. Sodium lauryl sulfate, known commercially as Gardinol or Duponol (trade names) is very effective. Also, sodium lauryl benzene sulfonate and certain of the free sulphonic acids, one of which is known commercially as Novonacco NN (trade name), are effective.

Where the amount of chromic acid present is not so high as to cause objectionable reaction, the use of alcohol is permissible. Tertiary butyl alcohol is among the least reactive and is therefore more preferable than some of the lower alcohols.

Although there is some difference in the efficiency of different wetting agents, .5% to 1% is usually sufficient. If alcohol is employed, amounts up to 5% or over may be required.

Numerous methods may be employed for the application of the treating solution. It is important in any event that the surface be uniformly wetted with the solution so that the etching will be uniform over the entire surface. The solution may be applied with a brush or by means of a spray gun, or the article can be momentarily dipped in a quantity of the solution.

After the wetting operation, the solution is allowed to dry upon the treated surface. The resulting film will contain iron phosphate, trivalent chromium and possibly some hexavalent chromium.

With the weaker solutions air drying is usually sufficient, but with higher concentrations it may be expedient to resort to a forced drying operation. After drying, the treated article is ready to be finished with paint, enamel, lacquer and so forth without further operations.

The following are examples of solutions that may be employed in carrying out the invention.

|       | Phosphoric acid | Chromic acid | Duponol (trade-mark) WA paste wetting agent |
|-------|-----------------|--------------|---------------------------------------------|
|       | Per cent        | Percent      | Percent                                     |
| No. 1 | 4.0             | .60          | .5                                          |
| No. 2 | 4.0             | .20          | .5                                          |
| No. 3 | 7.0             | 1.05         | .5                                          |
| No. 4 | 7.0             | .25          | .5                                          |
| No. 5 | 10.0            | 1.50         | .5                                          |
| No. 6 | 10.0            | .50          | .5                                          |

A specific example showing the use of the process is as follows: A cold rolled steel article is cleaned of oil and grease by wiping with naphtha and then drying the surface with clean cloths. A formula containing 10.0% phosphoric acid, 1.5% chromic acid, and .5% Duponol WA paste wetting agent is then applied to the surface by means of a brush. When the surface has been uniformly wetted the article is placed in an oven and dried for 3 minutes at 300° F. It is then removed and allowed to cool and is ready for the application of any desired paint finish without further treatment of the article.

If desired, the metal, the solution, or both may be heated prior to the rustproofing operation in order to facilitate the chemical action and hasten the drying.

Although many concentrations and many different proportions of the phosphoric acid and hexavalent chromium may be employed, in all cases it is necessary that the prevailing conditions shall allow etching of the ferrous surface to take place by the phosphoric acid present.

Any of the phosphorous acids may be substituted for the ortho-phosphoric acid. Among those are phosphorous acid, meta and pyro phosphoric acid, and hypo-phosphorous acid. The anhydrides, such as phosphorous pentoxide, can also be used since these materials immediately become acid upon addition to aqueous solution.

For the purpose of economy in shipping, the materials may be in concentrated form and diluted to the proper strength before use. In case it is desired to use a wetting agent or alcohol, it is best to add these after dilution since they will react with the chromic acid when in concentrated form.

The method of rustproofing according to this invention makes it possible to treat ferrous surfaces where it would be impractical with the usual coating procedure. The solutions can be used on stationary objects such as bridges, structural members of buildings, large oil tanks, truck bodies and so forth, there being no necessity for large immersion tanks or spray chambers. Heat can be dispensed with through the entire procedure which is impossible with the described phosphate methods. The resulting coating, however, compares favorably with the phosphate coatings when used as a paint base.

It is understood that the examples given above are merely illustrative and are not meant to limit the invention. The scope of the invention is to be measured only by the following claims.

We have discovered that in some instances the addition of a wetting agent to a solution containing chromic and phosphoric acids will cause the solution to etch the surface of the metal, whereas without the wetting agent, no etching would occur. The exact reason for this is not entirely clear but it is understood that such solutions, conditions, and coatings obtained in this way are within the scope of the invention.

What we claim is:

1. A ferrous metal object having on a surface thereof an integral coating having a composition resulting from drying onto said surface an aqueous solution containing phosphoric acid and chromic acid which will visibly etch the ferrous surface.

2. A ferrous metal object having on a surface thereof an integral coating having a composition resulting from drying onto the said surface an aqueous solution containing chromic acid and

phosphoric acid, the ratio between them being not more than .15 part of chromic for each part of phosphoric.

3. The method of producing a corrosion-resistant paint-holding coating integral with the metallic surface which comprises drying onto a ferrous surface an aqueous solution containing chromic acid and phosphoric acid which will visibly etch the ferrous surface.

4. The method of producing a corrosion-resistant paint-holding coating integral with the metallic surface which comprises drying onto a ferrous surface a film of an aqueous solution containing chromic acid and phosphoric acid, in which the ratio of chromic to phosphoric is not more than .15 to 1.

ROBERT R. TANNER.

ROBERT V. HARRIS.